

Jan. 31, 1967

S. COPPIK ET AL

3,301,745

PULP PROCESSING METHOD FOR MIXED CELLULOSIC MATERIALS

Filed April 26, 1963

3 Sheets-Sheet 1

Fig. 1



Jan. 31, 1967

S. COPPIK ET AL

3,301,745

PULP PROCESSING METHOD FOR MIXED CELLULOSIC MATERIALS

Filed April 26, 1963

3 Sheets-Sheet 2



Fig. 2



Fig. 3

INVENTORS  
SYDNEY COPPIK  
RALPH BROWN

BY

*Fred A. G...*

AGENT

Jan. 31, 1967

S. COPPIK ET AL

3,301,745

PULP PROCESSING METHOD FOR MIXED CELLULOSIC MATERIALS

Filed April 26, 1963

3 Sheets-Sheet 3



Fig. 4



Fig. 5



INVENTORS  
SYDNEY COPPIK  
RALPH BROWN

BY

*Fred A. Karr*

AGENT

Fig. 6

## 1

3,301,745

## PULP PROCESSING METHOD FOR MIXED CELLULOSIC MATERIALS

Sydney Coppick, Ridley Park, Pa., and Ralph Brown,  
Glastonbury, Conn., assignors to Scott Paper Company,  
Philadelphia, Pa., a corporation of Pennsylvania  
Filed Apr. 26, 1963, Ser. No. 275,857  
4 Claims. (Cl. 162—55)

This invention pertains to a novel method of pulp and paper utilization, more specifically, this invention involves a novel method of operating pulp and paper mills, as well as pulp converting facilities, designed to process pulp and produce papers of various kinds from mixed sources of cellulose containing materials and cellulose containing growth species pulped according to different pulping techniques.

The prior art pulp to paper processes, wherein the pulp was cooked according to the various techniques, produced pulps having characteristics of the species of wood cooked or the aggregate characteristics of the various species cooked. If the pulp to paper method incorporated pulp obtained from different processes, such as, kraft or sulfate and the sulfite, the composite characteristics of the two pulps often had unwanted properties in the final paper product. Consequently, heretofore, papers of various qualities and types had to be tailored starting with the wood species, the cooking process, the processing of pulps, such as, beating, bleaching, thickening and washing, and finally the paper sheet forming. Moreover, the prior art wood species to final paper route was predicated upon the use of the type of wood or cellulose containing material and the pulping and processing had to be tailored for the desired end result.

The present invention is an improvement in the cellulose containing material pulp to paper route in that the novel process allows great variation in the use of the cellulose containing material species and mixtures of species in the pulp to paper route. According to the present process, significantly greater pulp and paper processing latitude is achieved, not only in the type of cellulose containing material or wood or species of wood mixtures to be used, but also in the pulping and pulp processing operations, as well as in the final tailoring of the various papers desired.

The present invention is accomplished by a novel method of operating a cellulose pulping to paper web producing route comprising the steps of:

- (A) processing at least one species of cellulose containing material to be pulped in at least one type of pulping process;
- (B) pulping the cellulose containing material according to at least one pulping process in at least one pulping zone;
- (C) obtaining a screened pulp from said pulping zone;
- (D) separating the various fractions of said cooked and screened pulp by means capable of separating pulp fractions:
  - (1) the separating step being characterized by:
    - (a) separating a fraction of the screened pulp in a first pulp fraction separating zone,
    - (b) taking the first fraction and processing it for a first cellulose web producing zone,
    - (c) taking the remainder of the pulp stream and processing it to at least one subsequent pulp fraction removing zone having optional recycle streams, and having at least one final reject stream,
    - (d) taking at least one of the subsequent fraction streams and processing it for at least one additional cellulose web producing zone;

## 2

(2) said separating step being characterized by the selected pulp fraction possessing the selected different physical and chemical properties when said pulp fraction is further subjected to subsequent pulp processing steps;

(3) said separating step being further characterized by the said selected pulp fraction possessing the selected properties when said pulp fraction is incorporated in the final paper web;

(E) the pulp fraction separating step being readjusted according to the operating conditions of said pulp processing route; and

(F) the pulp fraction separating step being readjusted in combination with the pulp processing route according to the selected properties desired in the paper web.

In order to accomplish the most effective separating of the pulp fractions, as well as the operation of pulp processing and papermaking route, liquid cyclone means are used in practicing the invention. Liquid cyclones, such as, centricleaners, are suitable, other cyclones are equally efficient, however, in all cases, the reject orifices of the cyclones must possess means that may be changed to allow a gradation of opening sizes to permit the ready adjusting of the varying conditions and demands in the pulp processing and papermaking route.

The present invention is further accomplished by a continuous pulp to paper web producing route comprising the steps of:

(A) taking a screened pulp comprising of at least one species of wood pulped by at least one pulping process, containing various fractions of pulp having different chemical and physical properties;

(B) separating the various fractions of said screened pulp by means capable of separating pulp fractions;

(1) the separating step being characterized by:

(a) separating a fraction of the screened pulp in a first pulp fraction separating zone,

(b) taking the first fraction and processing it for a first cellulose web producing zone,

(c) taking the remainder of the pulp stream and processing it to at least one subsequent pulp fraction removing zone having optional recycle streams, and having at least one final reject stream,

(d) taking at least one of the subsequent fraction streams and processing it for at least one additional cellulose web producing zone;

(2) said separating step being characterized by the selected pulp fraction possessing the selected different physical and chemical properties when said pulp fraction is further subjected to subsequent pulp processing steps;

(3) said separating step being further characterized by said pulp fraction possessing the selected properties when said pulp fraction is incorporated in the final paper web;

(C) the pulp fraction separating step being readjusted according to the operating conditions of said pulp processing route when said route is changed by the varying pulp fractions being obtained from different sources of screened pulp in step (A);

(D) the pulp fraction separating step being readjusted in combination with the pulp processing route according to the selected properties desired in the paper web.

The invention as accomplished above is further amplified that in the method, the separating step, characterized by the pulp processing properties, is operated producing pulp fractions of same bleachability; and the separating

step is further characterized by the final paper web product of the first paper producing route being of improved strength and printing characteristics, and the final paper web product of a second paper web producing route being of improved softness, hand feel and absorbency.

The present invention is still further accomplished by a novel continuous method of operating a pulp to paper web producing route comprising the steps of:

(A) pulping at least one species of cellulose containing material possessing various fractions of cellulose pulp of different chemical and physical properties associated with each species of cellulose containing material and its growth cycle;

(B) obtaining a screened pulp consisting of mixed fractions of pulp;

(C) separating the various fractions by:

(1) introducing the screened pulp in a first liquid means pulp fraction separating zone,

(2) taking a portion of pulp from the first liquid means pulp fraction separating zone for further pulp processing and use in a first paper web producing route,

(3) taking the remainder of pulp from the first liquid means pulp fraction separating zone and introducing said remainder into a second liquid means pulp fraction separating zone,

(4) taking a part of the second liquid means pulp fraction separating zone accept effluent obtained by:

(a) combining the accept effluent recycled to said second zone from a third liquid means pulp fraction separating zone accept effluent which, in turn, has been made up of a fourth liquid means pulp fraction separating zone accept effluent combined and introduced into the third zone with the reject effluent from said second liquid zone, and

(b) the said remainder of pulp from said first zone, and further processing this pulp and using it in a second paper web producing route;

(5) said first, second, third and fourth liquid pulp fraction separating zones being characterized by the obtained pulp fractions possessing the pre-selected differing physical and chemical properties when said pulp fractions are further subjected to subsequent pulp processing steps;

(6) the said first, second, third and fourth liquid pulp fraction separating zones being further characterized by said pulp fractions possessing the selected properties when said pulp fractions are incorporated in the final paper web.

The method above again may be modified to be adjusted according to the needs of the pulp processing and papermaking route as outlined above.

The invention, as accomplished immediately above, is further amplified that in the method, the separating step, characterized by the pulp processing properties, is operated producing secondary accept fraction containing a reduced amount of parenchyma cells in respect to the total amount of parenchyma cells present in the wood pulped, and requiring less bleach chlorine for given brightness level in respect to the bleach chlorine for the unfractioned pulp; and the separating step is further characterized by the final paper web product of the second paper producing route being of improved absorbency properties. Again, the variations outlined in respect to the different facets of the accomplished invention may be incorporated in the other variations outlined above. It is to be understood that the flexibility of the invention is in no way hampered by the particular route followed if the liquid cyclone means are readily adjustable to accomplish the corresponding variations in the operating conditions. Thus, it is understood that the liquid cyclone separating

means are fully responsive to the operating conditions both upstream and downstream of the process route.

In another aspect, this invention is accomplished by a novel continuous method of operating a pulp to paper web producing route comprising the steps of:

(A) pulping at least one species of cellulose containing material possessing various fractions of cellulose pulp of different chemical and physical properties associated with each species of cellulose containing material and its growth cycle;

(B) obtaining a screened pulp consisting of mixed fractions of pulp;

(C) separating the various pulp fractions by:

(1) introducing the screened pulp into a first liquid means pulp fraction separating zone,

(2) taking a portion of a pulp fraction from the first liquid means pulp fraction separating zone and combining it with the accept fraction from a second liquid means pulp fraction separating zone for further pulp processing and use in a first paper web producing route,

(3) taking the reject fractions from the second liquid zone and introducing said fractions into the third liquid means pulp fraction separating zone,

(4) taking a portion of a pulp fraction from the third liquid means pulp fraction separating zone and combining it with the accept fractions from the fourth liquid means pulp fraction separating zone for further pulp processing and use in a first paper web producing route,

(5) taking the reject fraction from the third liquid zone and introducing said fraction into the said fourth liquid means pulp fraction separating zone,

(6) said first, second, third and fourth liquid pulp fraction separating zones being characterized by the obtained pulp fractions possessing the pre-selected differing physical and chemical properties when said pulp fractions are further subjected to subsequent pulp processing steps,

(7) the said first, second, third and fourth liquid pulp fraction separating zones being further characterized by said pulp fractions possessing the selected properties when said pulp fractions are incorporated in the final paper web.

In still another aspect, this invention may be accomplished by a novel continuous method of operating a pulp to paper web producing route comprising the steps of:

(A) pulping at least one species of cellulose containing material possessing various fractions of cellulose pulp of different chemical and physical properties associated with each species of cellulose containing material and its growth cycle;

(B) obtaining a screened pulp consisting of mixed fractions of pulp;

(C) separating the various pulp fractions by:

(1) introducing the screened pulp into a first liquid cyclone means pulp fraction separating zone,

(2) taking a portion of a pulp accepts fraction from the first liquid cyclone means pulp fraction separating zone and combining it with the accepts fraction from a second liquid cyclone means pulp fraction separating zone, wherein said second zone further is separating the rejects from said first zone, and using the two combined fractions for further pulp processing and use in a first paper web producing route,

(3) taking the reject fraction from the second zone and introducing said fractions into a third liquid cyclone means pulp fraction separating zone wherefrom the tertiary accepts are used for further pulp processing and use in a second paper web producing route,

(4) taking the reject fractions from the third zone and introducing said fraction into a fourth liquid cyclone means pulp fraction separating

zone wherefrom the quaternary accepts are used for further pulp processing and use in a third paper web producing route,

- (5) said first, second, third and fourth liquid pulp fraction separating zones being characterized by the obtained pulp fractions possessing the pre-selected differing physical and chemical properties when said pulp fractions are further subjected to subsequent pulp processing steps,
- (6) the said first, second, third and fourth liquid pulp fraction separating zones being further characterized by said pulp fractions possessing the selected properties when said pulp fractions are incorporated in the final paper web.

With the foregoing in mind, the present invention can be comprehended more readily by reference to the attached drawings wherein the same reference characters are used to indicate the corresponding zones and streams and wherein:

FIGURE 1 illustrates as an example of the invention, the diagrammatic flow sheet of the disclosed operation;

FIGURE 2 illustrates as an aspect of the invention another diagrammatic flow sheet of the liquid means pulp fraction separating zone;

FIGURE 3 illustrates as an aspect of the invention a still further diagrammatic flow sheet of the liquid means pulp fraction separating zone depicting thereby the various fraction separating arrangements possible;

FIGURE 4 depicts a mix of fibers in southern pine, magnified 950 times and containing springwood and summerwood;

FIGURE 5 depicts a fraction of southern pine magnified 950 times and containing a predominant portion of summerwood;

FIGURE 6 depicts a fraction of southern pine magnified 950 times and containing a predominant portion of springwood.

In reference to FIGURE 1, the novel process is carried out as follows: Area 1 represents the holding zone of cellulose containing material, such as, chips, straw, bagasse, or other known pulp yielding cellulose containing material. These materials are prepared according to the peculiar practices required for each species of starting material, as well as the type of pulping process used.

Area 2 represents another holding zone containing a species of cellulose containing material different from the material in Area 2. Of course, Areas 1 and 2 can represent holding zones having the same type of cellulose starting material. The digester 3 represents the pulping operation generally associated with either one or two stage sulfite operation or the kraft operation. The blow-pit 4 represents a generally well-known step in any pulping operation and so does the knot removing zone 5. The washing zone 6 likewise depicts the final liquor removing step. The washed pulp is then introduced into a washed pulp holding zone 7 from which the pulp is subjected to the screening operation 8, well-known in the art. The screening operation is used to separate the unacceptable contaminants. Generally, these screening operations are insufficient for some types of paper and the pulp must be further refined in order to remove the contaminants. Most prior art pulp mills have resorted to water cyclones to separate the final rejects from the pulp after the pulp has been screened. Consequently, dirt, shives and pitch particles often are removed by further processing of the screened pulp accumulated in a holding or storage zone, such as, 9.

However, in the present process, as depicted in FIGURE 1, liquid separating means I°, II°, III° and IV° (such as, cyclones, continuous centrifuges, or other separating means designed to take advantage of physical properties of pulp) are used to effect an integral function in the novel process in an entirely different manner, than previously used in the art. In the present process,

the preferred liquid cyclone separating means are used to obtain the natural, mechanical and chemical fractions of the pulp to separate the fractions according to their properties and to use the pulp fractions most suited for particular pulp processing steps or most suited as pulp material for papers having the particular paper properties associated with the particular pulp fraction.

In practicing the invention, the pulp fractions are separated by regulating the pressure of inlet water in the cyclone, the water velocity and the orifice opening. The particular combination of conditions which gives the desired result is found by test or trial runs for a given mix of cellulose starting materials or a given mix of pulp obtained from various sources. The important fact is that the pulp fractions as run are adjusted to suit the most economical and efficient operation of the mill to give the desired or pre-selected end results, which the varying pulp fractions afford because of their physical and chemical properties associated with the cellulose material and its growth cycle. By the same token, the novel method allows the use of a mixture of pulps in an optimum manner as well as the optimum use of each individual pulp fraction as it suits a certain pulp processing route or certain paper producing route.

Further, in reference to FIGURE 1 and the liquid separating means I°, II°, III°, and IV°, it is obvious that various arrangements may be used to obtain the proper mix of fractions suitable for particular uses. For example, additional liquid means may be used in series or in parallel with various recycle arrangements. The particular arrangement may give highly refined pulp fractions directed to particular end uses in specialty papers. The various arrangements may also separate fractions which may be highly desirable for use in printing papers, while the remaining functions may be processed without additional steps and used in bag or kraft papers.

Obviously, the operating flexibility, the optimum use of the pulp and wood, and the pulping chemicals are only some of the facets of this invention which characterize the novel process.

The primary pulp accepts in FIGURE 1 designated as stream A are further processed in the thickener 11e designated as thickener A and bleacher 12a designated as bleacher A. The pulp fraction, after the bleaching step, possesses different chemical properties and thus reacts differently under identical pulp processing conditions. Some of this and other pulp fraction behavior is further illustrated by the examples. The other processing steps, such as, washing 13, are self-explanatory and the particular operation of a paper machine 14 is also self-explanatory. However, it is important to understand that the operation of the paper machines will be different if the pulp fraction separating step will produce pulp fractions that have properties which do not require particular steps heretofore associated with the presently used mixed fraction pulps.

FIGURE 2, thus, shows a further arrangement of the liquid means for separating pulp fraction. The primary, secondary, tertiary and quaternary accepts produce a source of starting pulp material for the use in further pulp processing and final paper web producing routes designated as streams A and B respectively. Example V shows this particular operation.

FIGURE 3 again depicts a particular cyclone arrangement with the pulp fractions being separated into three streams for use in the various pulp processing steps and paper web making operations associated with the utilization of the particular pulp fractions. Example VIII further illustrates this particular operation.

FIGURE 4 depicts a collection of actual pulp fractions consisting of flat, flexible, predominantly ribbon-like springwood 1a; and 1b represents the rod-like, stiff summerwood fibers. The figure is a reproduction from a photograph of sample fibers taken from a representative batch of unfractionated southern pine pulp. The fibers

are oriented under a microscope and embedded lengthwise in it. The solidified polymer is then transferred to the microtome and cross-sections of the fiber strands are cut transversally across the axis and photographed with a reproduced magnification of 950 times.

FIGURE 5 depicts a collection of fibers in an actual pulp fraction used in the novel method. This fraction consists of predominantly rod-like, stiff summerwood fibers, designated as 1b and having most of springwood 1a removed. FIGURE 5 is obtained according to the same procedure used in obtaining the mixed fraction depicted in FIGURE 4. The fibers in FIGURE 5 have been magnified 950 times.

FIGURE 6 depicts a collection of pulp fibers in an actual pulp fraction used in the novel method. This fraction consists of predominantly ribbon-like, flexible, large surface area springwood fibers, designated as 1a and having most of the summerwood 1b fraction removed from the mixed starting pulp. The fibers in FIGURE 6 have been magnified 950 times and photographed as in FIGURE 4.

Other wood cells, such as, parenchyma cells, are likewise separated from the desired pulp fractions and the pulp fractions are used for their pre-selected purpose. By the same token, the novel method also incorporates the use of pulp fractions of fibers of different lengths or different geometrical configuration, as well as different chemical properties. For example, mixed and pulped species of wood, such as, a mixture of:

*Picea glauca*: Canadian Spruce  
*Picea mariana*: Black Spruce

*Pinus banksiana*: Jack Pine

*Tsuga canadensis*: Eastern Hemlock

*Populus tremuloides*: Quaking Aspen

*Populus grandidentata*: Bigtooth Aspen

contains a mixture of anatomic constituent cells having the following representative pulp fractions:

Springwood tracheids } from the conifers  
Summerwood tracheids }

Springwood vessels

Summerwood vessels } from the hardwoods  
Springwood fibers }

Summerwood fibers }  
Longitudinal parenchyma } from the conifers  
Radial parenchyma } and hardwoods.

The appended examples more fully illustrate the process and are intended only to illustrate but not to limit the present invention.

#### EXAMPLE I

In a pulp and papermaking operation producing simultaneously a strong tabulating grade of paper and a soft tissue grade on two different paper machines, the fractional fiber geometrical system was operated with respect to FIGURE 1, as follows:

Northeastern softwoods 1 (spruce and balsam fir) and northeastern hardwoods 2 (beech, birch and maple) were cooked together in an acid sulfite pulping digester 3 in the proportions of four parts of softwood to one part of hardwood.

On completion of the digestion, the combined delignified fibers were discharged to blow-pit 4 and the residual knots removed at 5. The deknotted pulp was washed free from spent cooking liquor on washer 6, and substantially freed from fiber bundles, shives, small splinters and residual bark by a series of screens 8 to produce screened pulp 9.

The screened pulp at 0.5% consistency was pumped through a series of liquid cyclones 10 arranged as in FIGURE 1 with the primary accepted stock separated to stream A. The primary rejected stock was fed to the secondary cyclones together with accepted stock recycle from the tertiary cyclones. The rejected stock from the tertiary

cyclones was fed to the quaternary cyclones and the quaternary accepted stock recycled to the feed of the tertiary cyclones. The final rejects from the quaternary cyclones, containing dirt particles, small bark specks and residual wood shives, which constituted 1.27% of the original stock, was discarded. The secondary accepted pulp was directed to stream B.

The cyclones were 3-inch maximum periferal diameter, and operated with 45 p.s.i.g. feed inlet pressure and 5 p.s.i.g. accept outlet pressure, with a flow of 30 gallons/minute for each cyclone. The reject tip orifices of the cyclones was  $\frac{1}{8}$  inch, so that the reject rate of the primary cleaners was about 20% of the feed rate. The flow rates and pressures of the subsequent stages were adjusted such that the final rejects from the fourth stage containing inorganic dirt, shives and bark particles were directed to the sewer and constituted 1.27% by weight of the primary feed pulp.

The production and pulp analysis data is shown in Table I. It is apparent that pulps of entirely different fiber characteristics are produced with regard to fiber length, hardwood content and proportions of spring and summerwood fibers, but with the same bleachability (permanganate number).

The pulp from stream A was directed to a paper machine producing tabulating card stock where paper was prepared with improved strength and printing characteristics, while that from stream B was directed to a tissue machine manufacturing creped towel with improved softness, handfeel and absorbency.

The fiber length fractionation data was obtained via the Bauer McNett method as per TAPPI standards.

TABLE I

| 35 | Unbleached                            |             | Bleached |          |
|----|---------------------------------------|-------------|----------|----------|
|    | Thickener A                           | Thickener B | Washer A | Washer B |
| 40 | 14 Mesh, Fraction Percent--           | 22.6        | 9.4      | 21.4     |
|    | 28 Mesh, Fraction Percent--           | 26.1        | 25.0     | 27.2     |
|    | Hardwood, Percent--                   | 22.9        | 30.1     | 27.9     |
|    | Pulp Production, tons/hour--          | 11.4        | 2.7      | -----    |
|    | Percent of Total Pulp--               | 80.9        | 19.1     | -----    |
|    | Permanganate No--                     | 13.4        | 13.4     | -----    |
|    | Brightness (photo-volt)--             | -----       | 79       | 86       |
| 45 | Ratio, Summerwood/Springwood Fibers-- | 1:1.47      | 1:1.25   | 1:1.73   |
|    |                                       |             |          | 1:1.18   |

#### EXAMPLE II

In another sulfite pulp and paper operation similar to Example I, the chip proportions fed to the digester were changed such that the wood blend contained about 30% hardwood. The operation was conducted as in Example I and depicted in FIGURE 1. The results were as follows:

TABLE II

| 55 | Pulp Analysis               | Screened Pulp Operation 9, Figure 1 |             | Unbleached Pulp From-- |             |
|----|-----------------------------|-------------------------------------|-------------|------------------------|-------------|
|    |                             | Thickener A                         | Thickener B | Thickener A            | Thickener B |
| 60 | 28 Mesh Fraction, percent-- | 26.1                                | 13.1        | 30.7                   | -----       |
|    | 14 Mesh Fraction, percent-- | 23.2                                | 28.4        | 24.7                   | -----       |
|    | Permanganate No--           | 12.1                                | 13.2        | 11.7                   | -----       |
|    | Hardwood, percent--         | 28.0                                | 34.0        | 22.5                   | -----       |

65 It is further apparent from the above that the pulp has been separated into streams with widely differing fiber characteristics. For example, the chlorine demand of stream A is different from the chlorine demand of stream B. This property of the pulp fraction is useful in adjusting the operating conditions of the pulp processing as well as the papermaking route.

#### EXAMPLE III

In a sulfite operation employing 25% hardwood and 75% softwood similar to that of Example II, the pulp

was separated into streams A and B as in FIGURE 1. The results were as follows:

TABLE III

| Pulp                                     | Freeness | Fraction percent |         |         |          |               |
|------------------------------------------|----------|------------------|---------|---------|----------|---------------|
|                                          |          | 14 Mesh          | 28 Mesh | 48 Mesh | 150 Mesh | Thru 150 Mesh |
| Screened Pulp (Operation 9, Fig. 1)----- | 644      | 22.0             | 34.4    | 16.8    | 19.3     | 7.5           |
| Stream A Pulp:                           |          |                  |         |         |          |               |
| From Thickener A-----                    | 655      | 20.6             | 34.3    | 15.5    | 16.2     | 13.4          |
| From Bleacher A-----                     | 628      | 23.5             | 38.2    | 13.6    | 18.0     | 6.7           |
| Stream B Pulp:                           |          |                  |         |         |          |               |
| From Thickener B-----                    | 687      | 3.8              | 35.0    | 23.0    | 23.6     | 14.6          |
| From Bleacher B-----                     | 621      | 7.3              | 40.1    | 16.7    | 29.9     | 1.0           |

It is apparent that at essentially the same freeness, the two pulps A and B have entirely different fiber length characteristics. In stream A, there is a wide distribution of long, medium and short fibers; while in stream B, the fibers are predominantly of the medium length varieties.

## EXAMPLE IV

In a Mitscherlich type acid sulfite pulping operation similar to that depicted in FIGURE 1, a single hardwood species; i.e., "populus tremuloids," was digested and the pulp processed as in Example I to produce the screened pulp. This stock was pumped at 0.5% consistency to the 3-inch primary liquid cyclones equipped with a  $\frac{1}{2}$  inch reject discharge orifice, such that the accepts constituted about 10% by weight of the feed, while the primary rejects contained the remaining 90% of the feed stock. These primary rejects were processed through three further stages of liquid cyclones as in Example I, with recycle as shown in FIGURE 1. The secondary, tertiary and quaternary cyclones were equipped with  $\frac{1}{8}$  inch reject orifices as in Example I, to culminate finally with a waste reject discharge of dirt and shives of 1.4% of the original pulp.

The primary accepted pulp of stream A was processed as in FIGURE 1, and utilized for a component of a paper-making furnish to produce a packaging grade of paper. The secondary accepted stock of stream B was processed separately as in FIGURE 1 to produce a pulp which was utilized as the major component in a soft absorbent tissue.

The properties of the predominant fraction are compared with those of the whole pulp in Table IV. It was noted by microscopical examination of the B stream that a substantial reduction in the number of radial parenchyma cells had taken place during the cyclone fractionation, and were present predominantly in the stream A. Moreover, on staining with Sudan II (manufactured by The Matheson Company, Inc., East Rutherford, New Jersey) and examining microscopically, it was observed that the pitch was for the most part contained within these radial parenchyma cells.

TABLE IV

| Pulp Quality                                                  | Unbleached Pulp From-----             |                        |
|---------------------------------------------------------------|---------------------------------------|------------------------|
|                                                               | Screened Pulp (Operation 9, Figure 1) | Thickener B (Figure 1) |
| Production Rate, percent of Total-----                        | 100                                   | 91.2                   |
| Pitch, percent-----                                           | 1.34                                  | 0.88                   |
| Chlorine Demand for 81 Brightness, lbs. available Cl/ton----- | 93.0                                  | 65.1                   |
| Aged Absorbency (seconds)-----                                | 377                                   | 241                    |

This is substantiated in Table IV, where the pitch, by alcohol-benzene extraction, is considerably reduced in stream B, with a corresponding improvement of the aged absorbency characteristics. These data were obtained by the accelerated aging of the paper sheets for 10 minutes at 300° F. and determining the time in seconds for the

complete absorption of 0.1 cc. of water added to the surface of the sheets as per TAPPI specifications. It is to be noted also that the bleaching requirements have been changed by the cyclone fractionation.

## EXAMPLE V

In another Mitscherlich acid sulfite pulping operation similar to Example IV, midwestern poplar wood was pulped and processed to screened pulp as in FIGURE 1. Thereafter, the pulp was fractionated in a series of liquid cyclones arranged as in FIGURE 2.

The cyclones were 3-inch diameter and operated with a  $\frac{1}{2}$ -inch reject discharge orifice to produce the fractional proportions of Table V.

The primary and secondary accepts were combined to produce stream A (FIGURE 2) while the tertiary and quaternary accepts were combined to form stream B of FIGURE 2.

Stream A was thickened, bleached and washed as in FIGURE 1 and fed as a component furnish to a paper machine producing a "wax base" stock for the manufacture of wax paper, while stream B was separately processed as in FIGURE 1 to produce a component of a furnish for a paper machine producing tissue stock for paper dinner napkin manufacture.

It is apparent from the data of Table V that the absorbency characteristics of the fractions constituting stream B are greatly improved over those of the original pulp. Moreover, the fractions constituting stream A were observed microscopically to contain the majority of the radial parenchyma cells containing resinous materials which contributed to the water resistant characteristics of this pulp stream and accordingly directed its advantageous use in wax base stock paper.

TABLE V

| Pulp From-----               | Percent of Total Feed | Aged Absorbency (seconds) |
|------------------------------|-----------------------|---------------------------|
| Primary Accepts-----         | 11.2                  | >1,200                    |
| Secondary Accepts-----       | 57.4                  | 580                       |
| Tertiary Accepts-----        | 27.6                  | 160                       |
| Quaternary Accepts-----      | 2.0                   | 45                        |
| Feed (from Operation 9)----- | 100                   | 480                       |
| Final Rejects to Sewer-----  | 1.8                   | -----                     |

## EXAMPLE VI

In an alkaline pulping operation of the kraft or sulfate type, southern pine was pulped, deknotted, washed and screened as in FIGURE 1. The pulp was then fractionated through a series of liquid cyclones as in Example V according to the arrangement of FIGURE 2. The primary and secondary accepts were combined to produce stream A while the tertiary and quaternary accepts were combined to produce stream B. These streams were thickened, bleached and washed as in FIGURE 1, and bleached stream A was directed as a component furnish to a paper machine producing a strong notion bag paper, while the bleached stream B was directed to a paper machine producing a printing grade of specialty paper.

It is obvious from the data of Table VI that the components of stream A contain a considerably larger proportion of long fibers than do those of stream B, and hence their papermaking characteristics are quite different.

TABLE VI

| Pulp From-----              | Percent of Total Feed | Bauer McNett, Fraction percent Retained on----- |         |         |          |
|-----------------------------|-----------------------|-------------------------------------------------|---------|---------|----------|
|                             |                       | 14 Mesh                                         | 28 Mesh | 48 Mesh | 150 Mesh |
| Feed from Operation 9-----  | 100                   | 69.4                                            | 16.6    | 8.0     | 6.0      |
| Primary Accepts-----        | 7.2                   | 83.5                                            | 8.9     | 3.8     | 3.8      |
| Secondary Accepts-----      | 54.8                  | 72.3                                            | 15.2    | 7.0     | 5.5      |
| Tertiary Accepts-----       | 31.5                  | 69.6                                            | 11.2    | 10.9    | 13.7     |
| Quaternary Accepts-----     | 5.5                   | 55.0                                            | 25.1    | 13.7    | 6.2      |
| Final Rejects to Sewer----- | 1.0                   | -----                                           | -----   | -----   | -----    |

## EXAMPLE VII

In a kraft sulfate operation pulping southern pine, the stock was processed according to the flow diagram of FIGURE 1. The reject orifice of the primary cyclone was  $\frac{1}{2}$  inch so that the primary accepts constituted 11.5% of the total feed.

Streams A and B were bleached and the A stream directed to a paper machine producing a glassine grade of paper, while stream B was directed to a paper machine producing mimeograph paper. The properties of the pulps are shown in Table VII.

TABLE VII

| Beating Time (minutes)  | Breaking Length (meters) |       |       |       |       |       |       |
|-------------------------|--------------------------|-------|-------|-------|-------|-------|-------|
|                         | 0                        | 5     | 15    | 25    | 35    | 45    | 60    |
| Pulp:                   |                          |       |       |       |       |       |       |
| Feed Pulp (Operation 9) | 3,500                    | 5,600 | 7,500 | 8,400 | 9,000 | 9,400 | 9,600 |
| Stream A                | 6,600                    | 8,400 | 8,800 | 9,300 | 9,500 | 9,700 | 9,900 |
| Stream B                | 3,200                    | 5,000 | 6,400 | 7,500 | 8,300 | 8,900 | 9,300 |

It is apparent from Table VII that the refining characteristics of the two pulps are entirely different. Stream A is an easy beating pulp with rapid strength development and resembles somewhat a sulfite pulp. However, stream B is a typical hard kraft pulp with particularly slow strength development. It is obvious that the papermaking qualities of these two pulps differ greatly. It is also obvious that these properties are useful in the pulp preparing, as well as papermaking process to adjust the processing conditions to achieve the most effective use of the various pulp fractions.

## EXAMPLE VIII

In a kraft operation digesting Georgia pine as in FIGURE 1, the screened pulp from operation 9 was processed through a series of liquid cyclones according to the flow diagram of FIGURE 3. The cyclones were 3-inch diameter and the primary, secondary units had  $\frac{1}{2}$ -inch reject orifices while the tertiary and quaternary units had a  $\frac{1}{8}$ -inch orifice. The inlet pressures to all of the cyclones were maintained at 40 p.s.i.g., the primary and secondary accepts were combined to produce stream A, the quater-

5

Bleached stream B was directed to the paper manufacture of a bag stock with particular stiffness qualities. Microscopical examination of the cross-section of the fibrous components of the original feed pulp in FIGURE 4 are compared with the cross-sections of the fibrous components in pulp fractions in streams A and B in FIGURE 6 and FIGURE 5, respectively.

The widely differing pulp characteristics are manifested in these photomicrographs and testify to the improved utility of this process for different papermaking purposes.

The original pulp contains a mixture of both springwood and summerwood fibers, stream A contains predominantly the ribbon-like, flexible, large surface area springwood fibers; while Stream B contains predominantly the rod-like, stiff summerwood fibers. The relative production rates of the various fractional components of these streams are shown in Table VIII.

TABLE VIII

| Pulp:                         | Percent of original feed |
|-------------------------------|--------------------------|
| Screened Pulp (Operation 9)   | 100                      |
| Primary Accepts               | 5.7                      |
| Primary Rejects               | 94.3                     |
| Secondary Accepts             | 6.1                      |
| Secondary Rejects             | 88.2                     |
| Tertiary Accepts              | 72.0                     |
| Tertiary Rejects              | 16.2                     |
| Quaternary Accepts            | 14.6                     |
| Quaternary Rejects (to sewer) | 1.6                      |

## EXAMPLE IX

Depithed bagasse was digested in a two stage alkaline pulping process, the first stage of which was similar to that depicted in FIGURE 1. After the first pulping stage, the partially digested fiber was screened as in FIGURE 1, and the insufficiently pulped screenings were subjected to a second stage alkaline digestion. The screened pulp from the first digestion stage was processed through a series of liquid cyclones as in FIGURE 1, with the primary cyclones equipped with  $\frac{1}{8}$ -inch reject orifices. Similar experimental fractionation runs were made with the primary reject orifice set at  $\frac{3}{16}$  inch and  $\frac{1}{4}$  inch. The results were as follows:

TABLE IX

| Primary Reject Orifice (inches) | Pulp From— | Percent Total Pulp | Bauer McNett Classification |                        | Freeness, cc. | Breaking Length, meters | Spec. vol., cc./gr. | Mullen, lb. |
|---------------------------------|------------|--------------------|-----------------------------|------------------------|---------------|-------------------------|---------------------|-------------|
|                                 |            |                    | On 150 Mesh, percent        | Thru 150 Mesh, percent |               |                         |                     |             |
| $\frac{1}{16}$                  | Stream A   | 57.4               | 54.8                        | 45.2                   | 104           | 5,604                   | 1.38                | 18.5        |
|                                 | Stream B   | 42.6               | 77.4                        | 22.6                   | 596           | 2,435                   | 2.00                |             |
| $\frac{3}{16}$                  | Stream A   | 50.8               | 68.5                        | 31.5                   | 119           | 4,031                   | 1.60                | 10.0        |
|                                 | Stream B   | 49.2               | 84.3                        | 15.7                   | 549           | 2,268                   | 2.18                |             |
| $\frac{1}{4}$                   | Stream A   | 37.7               | 48.0                        | 52.0                   | 67            | 4,433                   | 1.41                | 19.0        |
|                                 | Stream B   | 62.3               | 86.0                        | 14.0                   | 498           | 2,530                   | 1.80                |             |

nary accepts formed stream B, while the tertiary accepts formed stream C.

Each of these streams was processed separately as in FIGURE 1 to result in three pulps, two entirely different; i.e., streams A and B and a third intermediate pulp, stream C, somewhat similar in properties to the whole original pulp.

Streams A and B were bleached separately, while stream C was processed unbleached and utilized for the production of a brown wrapping paper.

Bleached stream A was directed to a paper machine and utilized as a component of a furnish producing a grade of offset paper with particular printing qualities such that fiber flexibilities enhanced the surface bonding of the sheet and reduced substantially the collection of fibers transferred from the sheet to the printing rolls.

60

It is again apparent that the process has separated the original pulp into two streams with entirely different fiber lengths, drainage characteristics, strengths and bulks. Stream A was utilized as a component in a papermaking furnish for corrugated packaging media, while stream B was used in a paperboard for impregnating purposes.

## EXAMPLE X

Another run was made of a 0.5% consistency slurry of southern kraft pine with three hydrocyclones arranged in series. The reject orifices for the respective primary, secondary and tertiary cyclones were adjusted to  $\frac{1}{2}$  inch,  $\frac{1}{4}$  inch and  $\frac{1}{8}$  inch and were used to obtain four pulp fractions. TAPPI handsheets were made of the starting feed and the four fractions. The different pulps gave the following results:

TABLE X

| Sample          | Percent of Feed | Freeness, cc. | Breaking Length, meters | TAPPI Tear Factor | Mullen, lb. | Spec. vol., cc./g. | Bauer-McNutt |      |      |
|-----------------|-----------------|---------------|-------------------------|-------------------|-------------|--------------------|--------------|------|------|
|                 |                 |               |                         |                   |             |                    | 14%          | 28%  | 48%  |
| Feed            |                 | 740           | 3,520                   | 178               | 18.0        | 1.91               | 69.3         | 16.6 | 8.0  |
| 1st run Accepts | 7.2             | 580           | 6,680                   | 188               | 40.3        | 1.62               | 83.5         | 8.9  | 3.8  |
| 2nd run Accepts | 54.8            | 690           | 3,280                   | 178               | 19.5        | 1.83               | 72.4         | 15.2 | 7.0  |
| 3rd run Accepts | 31.5            | 729           | 3,240                   | 138               | 14.0        | 1.94               | 69.6         | 11.2 | 11.2 |
| 3rd run Rejects | 6.5             | 747           | 2,670                   | 117               | 11.9        | 2.00               | 55.0         | 25.1 | 13.7 |

From the above data, it is obvious that pulps of different characteristics may be processed at different conditions before the pulps are used in a papermaking machine. The data also show that the same species of wood yields pulps having entirely different properties and uses. Moreover, the high throughput operations commonly encountered in pulp and paper mills are compatible with the present invention as any size of mill can be converted to the novel method of operation.

#### EXAMPLE XI

##### A. Fractionation

Two runs were made in which a 0.5% consistency slurry of unbleached 80% northeastern softwood and 20% northeastern hardwood sulfite pulp was pumped through a 3-inch hydrocyclone. A  $\frac{5}{16}$ -inch diameter rejects nozzle produced a 69.6/30.4 accepts/rejects pulp fractions and a  $\frac{3}{8}$ -inch diameter nozzle produced a 54.6/45.4 accepts/rejects pulp fractions. Pulp fractionated in this manner was beaten in a Valley Beater to compare the strength levels of the two fractions. The results of TAPPI handsheets of these beater runs are given in Table XI.

C.C.S.F. and run to make an 18 lb./ream flat sheet. The properties of the paper are given in the following table.

TABLE XII.—MACHINE PAPER OF NORTHEASTERN 80% SOFTWOOD AND 20% HARDWOOD PULP FRACTIONS

|    |  |                                 | Accepts                  | Rejects     |
|----|--|---------------------------------|--------------------------|-------------|
|    |  |                                 | Percent of Original Pulp | 45.4        |
|    |  | C.C.S.F.                        | 449                      | 420         |
|    |  | Breaking Length (MD/CD), meters | 7,710/4,780              | 6,990/3,630 |
| 25 |  | Burst (Mullen), lbs.            | 12.8                     | 8.9         |
|    |  | TAPPI Tear Factor (MD/CD)       | 52/43                    | 44/38       |
|    |  | Specific Volume, cc./g.         | 1.36                     | 1.30        |
|    |  | Opacity, percent                | 45.1                     | 41.9        |
|    |  | Brightness, G.E.                | 76.0                     | 78.2        |
|    |  | Basis Weight, lbs./ream         | 18.8                     | 17.9        |

20 The paper machine run data show that the accepts pulp fraction gives a stronger sheet than the rejects pulp fraction with respect to breaking length, tear factor and Mullen even when both sheets are beaten to the same freeness. 35 The opacity of the accepts fraction is slightly more than that of the rejects. The brightness of the accepts is 2 points below that of the rejects due to the presence of larger amount of parenchyma cells which makes the pulp more difficult to bleach.

TABLE XI.—BEATER RUNS OF FRACTIONS OF UNBLEACHED PULP FROM 80% SOFTWOOD/20% HARDWOOD CHIPS  
RUN 1—69.6/30.4—ACCEPTS/REJECTS PULP FRACTION RATIO

| Beating Time (Minutes) | C.C.S.F.* |     | Breaking Length, meters |       | Mullen Factor, lbs. |      | TAPPI Tear Factor |    | Specific Volume, cc./g. |      | Basis Weight, g./M <sup>2</sup> |      |
|------------------------|-----------|-----|-------------------------|-------|---------------------|------|-------------------|----|-------------------------|------|---------------------------------|------|
|                        | A         | R   | A                       | R     | A                   | R    | A                 | R  | A                       | R    | A                               | R    |
| 0                      | 646       | 655 | 7,290                   | 6,978 | 34.7                | 33.8 | 111               | 96 | 1.35                    | 1.40 | 62.1                            | 63.7 |
| 3                      | 574       | 602 | 8,729                   | 7,519 | 37.8                | 35.5 | 93                | 88 | 1.32                    | 1.35 | 63.6                            | 62.1 |
| 6                      | 494       | 508 | 8,425                   | 7,999 | 39.3                | 36.5 | 78                | 79 | 1.27                    | 1.28 | 61.8                            | 63.4 |
| 9                      | 389       | 406 | 9,242                   | 8,095 | 42.8                | 39.0 | 67                | 76 | 1.20                    | 1.24 | 63.7                            | 61.4 |
| 12                     | 273       | 276 | 9,328                   | 8,359 | 43.5                | 40.5 | 63                | 67 | 1.15                    | 1.18 | 63.9                            | 62.4 |

RUN 2—54.6/45.4—ACCEPTS/REJECTS PULP FRACTION RATIO

|    |     |     |       |       |      |      |     |    |      |      |      |      |
|----|-----|-----|-------|-------|------|------|-----|----|------|------|------|------|
| 0  | 611 | 645 | 8,842 | 7,639 | 40.0 | 37.3 | 101 | 98 | 1.30 | 1.36 | 64.4 | 61.6 |
| 3  | 554 | 608 | 9,285 | 8,318 | 42.0 | 38.0 | 88  | 87 | 1.22 | 1.29 | 62.5 | 61.0 |
| 6  | 447 | 519 | 9,387 | 8,957 | 44.5 | 39.3 | 77  | 77 | 1.16 | 1.26 | 61.4 | 60.7 |
| 9  | 364 | 443 | 9,807 | 8,783 | 46.0 | 42.0 | 69  | 74 | 1.15 | 1.25 | 61.7 | 61.8 |
| 12 | 230 | 317 | 9,652 | 9,363 | 46.7 | 41.5 | 67  | 63 | 1.09 | 1.20 | 63.1 | 61.3 |

\*Canadian Standard Freeness, cc. A = Accepts Stream Fraction. R = Rejects Stream Fraction.

#### B. Paper machine runs

The two fractions obtained in the run with 54.6% accepts and 45.4% rejects were bleached and run under substantially identical conditions on a 10 paper machine. Both fractions were given a single stage hypochlorite bleach at 10% consistency with 100% chlorine demand and bleached to trace residual according to TAPPI standards. The two fractions were beaten to between 400–450

70 The above example illustrates how the pulp fraction separating step in the present invention is characterized by the conditions of the pulp processing stream as well as by the conditions in the paper machine run. The above example clearly teaches how the pulp fraction separating step may be used in conjunction with the desired conditions in the pulp processing stage and the papermaking stage or vice versa.

Further, from the above examples, it is readily apparent that the various chemical and physical properties of the pulp fractions may be used to adjust the operating rates, conditions and demands both upstream, e.g., in the chip preparing stages, digesting stages, etc., as well as downstream, e.g., the bleaching, beating and paper producing and also finally, in final paper product utilization. The flexibility obtained by the novel method is one of the improvements over the heretofore rather inflexible pulp and papermaking processes.

We claim:

1. A continuous method of operating a pulp to paper web producing route comprising the steps of:

- (A) pulping at least two species of cellulose containing material possessing various fractions of cellulose pulp of different chemical and physical properties associated with each species of cellulose containing material and its growth cycle, thereby obtaining a screened pulp consisting of mixed fractions of pulp;
- (B) separating the various fractions by:
  - (1) introducing the screened pulp in a first liquid means pulp fraction separating zone,
  - (2) taking a portion of pulp from the first liquid means pulp fraction separating zone for further pulp processing and use in a first paper web producing route,
  - (3) taking the remainder of pulp from the first liquid means pulp fraction separating zone and introducing said remainder into a second liquid means pulp fraction separating zone,
  - (4) taking a part of the second liquid means pulp fraction separating zone accept effluent obtained by:
    - (a) combining the accept effluent recycled to said second zone from a third liquid means pulp fraction separating zone accept effluent which, in turn, has been made up of a fourth liquid means pulp fraction separating zone accept effluent combined and introduced into the third liquid zone with the reject effluent from said second liquid zone, and
    - (b) the said remainder of pulp from said first zone and further pulp processing and use in a second paper web producing route;

- (5) said first, second, third and fourth liquid pulp fraction separating zones being characterized by the obtained pulp fractions possessing the pre-selected differing physical and chemical properties when said pulp fractions are further subjected to subsequent pulp processing steps;
- (6) the said first, second, third and fourth liquid pulp fraction separating zones being further characterized by said pulp fractions possessing the selected properties when said pulp fractions are incorporated in the final paper web.

2. A continuous method of operating a pulp to paper web producing route comprising the steps of:

- (A) pulping at least two species of cellulose containing material possessing various fractions of cellulose pulp of different chemical and physical properties associated with each species of cellulose containing material and its growth cycle, thereby obtaining a screened pulp consisting of mixed fractions of pulp;
- (B) separating the various pulp fractions by:
  - (1) introducing the screened pulp into a first liquid means pulp fraction separating zone,
  - (2) taking a portion of a pulp fraction from the first liquid means pulp fraction separating zone and combining it with the accept fraction from a second liquid means pulp fraction separating zone for further pulp processing and use in a first paper web producing route,
  - (3) taking the reject fractions from the second liquid zone and introducing said fractions into

the third liquid means pulp fraction separating zone,

- (4) taking a portion of a pulp fraction from the third liquid means pulp fraction separating zone and combining it with the accept fractions from the fourth liquid means pulp fraction separating zone for further pulp processing and use in a first paper web producing route,
- (5) taking the reject fraction from the third liquid zone and introducing said fraction into the said fourth liquid means pulp fraction separating zone,
- (6) said first, second, third and fourth liquid pulp fraction separating zones being characterized by the obtained pulp fractions possessing the pre-selected differing physical and chemical properties when said pulp fractions are further subjected to subsequent pulp processing steps,
- (7) the said first, second, third and fourth liquid pulp fraction separating zones being further characterized by said pulp fractions possessing the selected properties when said pulp fractions are incorporated in the final paper web.

3. A continuous method of operating a pulp to paper web producing route comprising the steps of:

- (A) pulping at least two species of cellulose containing material possessing various fractions of cellulose pulp of different chemical and physical properties associated with each species of cellulose containing material and its growth cycle, thereby obtaining a screened pulp consisting of mixed fractions of pulp;
- (B) separating the various pulp fractions by:
  - (1) introducing the screened pulp into a first liquid cyclone means pulp fraction separating zone,
  - (2) taking a portion of a pulp accepts fraction from the first liquid cyclone means pulp fraction separating zone and combining it with the accepts fraction from a second liquid cyclone means pulp fraction separating zone, wherein said second zone further is separating the rejects from said first zone and using the two combined fractions for further pulp processing and use in a first paper web producing route,
  - (3) taking the reject fraction from the second zone and introducing said fractions into a third liquid cyclone means pulp fraction separating zone wherefrom the tertiary accepts are used for further pulp processing and use in a second paper web producing route,
  - (4) taking the reject fractions from the third zone and introducing said fraction into a fourth liquid cyclone means pulp fraction separating zone wherefrom the quaternary accepts are used for further pulp processing and use in a third paper web producing route,
  - (5) said first, second, third and fourth liquid pulp fraction separating zones being characterized by the obtained pulp fractions possessing the pre-selected differing physical and chemical properties when said pulp fractions are further subjected to subsequent pulp processing steps,
  - (6) the said first, second, third and fourth liquid pulp fraction separating zones being further characterized by said pulp fractions possessing the selected properties when said pulp fractions are incorporated in the final paper web.

4. The method of claim 1 wherein the separating step (B), characterized by the pulp processing properties, is operated producing secondary accept fraction containing a reduced amount of parenchyma cells in respect to the total amount of parenchyma cells present in the wood pulped, and requiring less chlorine demand for given brightness level in respect to the chlorine demand for the unfractionated pulp; and the separating step is further characterized by the final paper web product of the sec-

3,301,745

17

ond paper producing route being of improved absorbency  
properties.

18

|           |         |          |       |          |
|-----------|---------|----------|-------|----------|
| 2,913,362 | 11/1959 | Cusi     | ----- | 162-55   |
| 2,972,171 | 2/1961  | Heritage | ----- | 162-55 X |
| 3,085,927 | 4/1963  | Pesch    | ----- | 162-55   |

**References Cited by the Examiner**

UNITED STATES PATENTS

1,809,312 6/1931 Richter ----- 162-55

5 DONALL H. SYLVESTER, *Primary Examiner.*

HOWARD R. CAINE, *Examiner.*